

# United States Patent Office

2,747,989

Patented May 29, 1956

1

2,747,989

## FERRITIC ALLOYS

**Henry William Kirkby and Charles Sykes, Sheffield, England, assignors, by mesne assignments, to Firth-Vickers Stainless Steels Limited, Sheffield, England, a British company**

No Drawing. Application April 1, 1953,  
Serial No. 346,257

Claims priority, application Great Britain May 28, 1952

**3 Claims. (Cl. 75—128)**

This invention relates to ferritic alloys and is concerned with the provision of forgeable high strength ferritic alloys possessing a good combination of strength and ductility coupled with stainless and (if required) non-scaling properties, without having recourse to the usual hardening and tempering processes.

Normally, high strength structural steels owe their characteristic physical properties to the peculiar relationship between the carbon and iron contents, which, in some cases, may be implemented by suitable alloying elements. With these steels, it is necessary for attainment of the desirable properties to submit them to thermal treatments comprising heating into the gamma (or austenitic) region, cooling at not less than a certain rate (e. g. air, oil or water cooled) followed by a tempering or letting down process to the required strength. Failure to use the appropriate hardening temperatures and cooling rates often leads to the material being too high in strength and low in ductility or vice versa.

A further difficulty in regard to the type of steel in question, is that where high chromium contents are used to impart rustless and scale-resisting properties it is necessary to use relatively higher hardening temperatures with consequent greater risks of warpage, loss of metal and/or spoiling of the surface appearance. This latter difficulty has a particular bearing in those cases where the article is required to meet close dimensional requirements such as with precision stamped articles.

such as with precision stamped articles.

This invention provides a ferritic alloy which does not rely on the element carbon and associated thermal treatments to impart the necessary strength, but upon the use of a selected critical balance of alloying elements with iron, which elements (each present within a critical range) collectively have a natural intrinsic hardness and strength.

The alloys according to the invention comprise the following range of composition:

|           |                            |
|-----------|----------------------------|
| Carbon    | Up to 0.1%.                |
| Silicon   | 1.5 to 6.0%.               |
| Manganese | 0.5 to 5.0%.               |
| Nickel    | 0.5 to 6.0%.               |
| Chromium  | 3.0 to 16.0%.              |
| Iron      | The substantial remainder. |

Niobium, titanium, vanadium or molybdenum, either singly or in combination, may be present in small quantities up to a total maximum of 1.0%.

The preferred range is:

|                     |               |
|---------------------|---------------|
| Carbon              | 0.1% maximum. |
| Silicon             | 2.0 to 5.0%.  |
| Manganese           | 2.0 to 4.0%.  |
| Nickel              | 3.0 to 6.0%.  |
| Chromium            | 8.0 to 14.0%. |
| Titanium or niobium | Up to 0.75%.  |
| Iron                | Remainder.    |

The following are examples of alloys embodying the invention and of their typical properties: 70

2

|              | C,<br>Percent | Si,<br>Percent | Mn,<br>Percent | Ni,<br>Percent | Cr,<br>Percent | Ti,<br>Percent | Nb,<br>Percent |
|--------------|---------------|----------------|----------------|----------------|----------------|----------------|----------------|
| Alloy A..... | 0.08          | 2.69           | 2.50           | 3.59           | 13.64          | -----          | 0.52           |
| Alloy B..... | 0.07          | 4.61           | 3.14           | 5.16           | 8.50           | -----          | -----          |
| Alloy C..... | 0.07          | 4.44           | 3.22           | 5.25           | 8.57           | 0.37           | -----          |

### Properties

|         | Yield point,<br>tons per<br>sq. inch | Maximum<br>Stress,<br>tons per<br>sq. inch | Elonga-<br>tion,<br>percent | Reduction<br>of<br>area,<br>percent | Izod<br>impact,<br>ft. lbs. |
|---------|--------------------------------------|--------------------------------------------|-----------------------------|-------------------------------------|-----------------------------|
| Alloy A | 49.0                                 | 65.0                                       | 24                          | 56                                  | 77                          |
| Alloy B | 62.0                                 | 84.5                                       | 20                          | 47                                  | -----                       |
| Alloy C | 54.8                                 | 83.0                                       | 21.5                        | 41                                  | -----                       |

20 The alloys of the invention are, for all practical purposes, unaffected by thermal treatments and consequently do not require hardening and tempering as is the case with the normal high strength ferritic alloys previously referred to. Where, however, cold work has been applied during fabrication, it may be necessary to employ a stress-relieving treatment, carried out at, say, 650-700° C. The following results of tests, carried out on alloys of the composition A referred to above, illustrate the non-sensitivity to heat treatment of the alloys of the present invention:

| Heat Treatment                         | 1 hour at 700° C.<br>and air-cooled from that temperature | 1 hour at 750° C.<br>and air-cooled from that temperature | Air cooled from 900° C. | Air cooled from 900° C. followed by 1 hour at 700° and air-cooled from that temperature |
|----------------------------------------|-----------------------------------------------------------|-----------------------------------------------------------|-------------------------|-----------------------------------------------------------------------------------------|
| Yield Point, tons per sq. inch-----    | 49.0                                                      | 51.0                                                      | 49.0                    | 50.0                                                                                    |
| Maximum Stress, tons per sq. inch----- | 65.0                                                      | 65.0                                                      | 67.5                    | 66.9                                                                                    |
| Elongation, percent-----               | 24                                                        | 19                                                        | 17                      | 21                                                                                      |
| Reduction of area, percent-----        | 56.0                                                      | 53.0                                                      | 51.5                    | 59.0                                                                                    |
| Izod Impact, ft. lbs-----              | 77                                                        | 86                                                        | 36                      | 84                                                                                      |

45 We claim:

1. A forgeable high strength ferritic alloy comprising carbon up to 0.1%, silicon 1.5 to 6.0%, manganese 0.5 to 5.0%, nickel 0.5 to 6.0%, chromium 3.0 to 16.0%, and the balance iron with residual impurities in ordinary amounts.

50 amounts.  
2. A forgeable high strength ferritis alloy comprising carbon up to 0.1%, silicon 1.5 to 6.0%, manganese 0.5 to 5.0%, nickel 0.5 to 6.0%, chromium 3.0 to 16.0%, up to 1.0% of an alloying constituent consisting of at 55 least one metal selected from a group consisting of niobium, titanium, vanadium, molybdenum and the balance iron with residual impurities in ordinary amounts

3. A forgeable high strength ferritic alloy comprising carbon up to 1.0%, silicon 2.9 to 5.0%, manganese 2.0 to 4.0%, nickel 3.0 to 6.0%, chromium 8.0 to 14.0%, up to 0.75% of a metal selected from the group consisting of titanium and niobium, and the balance iron with residual impurities in ordinary amounts

**References Cited in the file of this patent**

UNITED STATES PATENTS

2,225,730 Armstrong Dec. 24, 1940  
FOREIGN PATENTS  
625,055 France Aug. 2, 1927  
897,766 France Mar. 30, 1945